

## UNITED STATES PATENT OFFICE.

CARL ROBERT SCHROEDER, OF HOBOKEN, NEW JERSEY.

## METHOD OF PRODUCING METALS OR ALLOYS.

No Drawing.

Application filed November 22, 1919. Serial No. 339,905.

To all whom it may concern:

Be it known that I, CARL R. SCHROEDER, a citizen of the United States, and resident of Hoboken, in the county of Hudson and **5** State of New Jersey, have invented certain new and useful Methods of Producing Metals or Alloys, of which the following is a specification.

The invention relates to the reduction of **10** metals or metallic alloys from ores or compounds which are comparatively high in impurities which would be objectionable or deleterious to the metalliferous product, and has for its object to produce the desired metals **15** or alloys in relatively pure, or at least commercially acceptable condition, by so effecting the reducing reaction that the desired metalliferous values will be reduced selectively with respect to the impurities or **20** undesirable reducible elements, so that the latter will be practically eliminated or occur only in permissible amounts in the ultimate product. It has been found that by **25** properly regulating the quantity of the reducing agent, in accordance with the relative quantities or proportions of the desirable and undesirable elements occurring in the treated ores or compounds, the reducing reaction may be carried out in such manner **30** as to reduce the desired metal or alloy without effecting any material reduction of the undesired or objectionable components so that the latter will be either substantially eliminated from the ultimate product, or **35** will occur in such small proportions therein as to constitute no serious impairment of the commercial value of the ultimate metal or alloy.

In the production of metals from ores, **40** oxides or other compounds, by the reaction of a reducing agent, the oxygen of the ore or oxide combines with the reducing agent or some reactive elements thereof, and liberates the metal. When the reaction is produced by the aluminothermic method it has **45** always been found necessary, heretofore, in order to effect the production of the metals relatively low in impurities, that the ore or oxide used be also low in these impurities, **50** and it was usual, except in cases involving the use of rather pure natural ores and oxides, to purify the ores and oxides by one or more of the well known mechanical, metallurgical, or chemical methods, which

naturally required the expenditure of **55** considerable time and monetary cost, and was usually accompanied by loss in the quantity of the metallic values recovered. For example, in the manufacture of high percentage tungsten alloys by the aluminothermic process the success of the reaction required the employment of relatively pure and expensive raw material, or an artificially prepared tungsten compound in which the preparatory treatment was effected, at a **60** cost of time and money, to eliminate any undesirable elements or compounds which would impair the ultimate product. The conditions which apply to the production of metallic tungsten by the reduction process **65** also exist in the application of the process to the production of tungsten alloys, such as ferro-tungsten, from practically all kinds of tungsten ores, such as scheelite, wolframite, ferberite, and others, which nearly always contain such impurities as silicon, **70** manganese, phosphorus, sulphur, etc., which must be practically eliminated or reduced to such proportions that they will be innocuous in the ultimate ferro-tungsten alloy.

I have discovered that it is possible to control the proportions of the impurities in the final metalliferous product by a direct variation of the amount of the reducing agent employed, and while the invention finds particularly efficacious application to the reduction of metallic compounds by the aluminothermic method, it is not limited to such method, but is applicable to other reducing reactions in which the quantities of **75** the reducing agent can be controlled and regulated in accordance with the proportions of the desired metallic values occurring in the compounds treated, the reactions occurring by what may be termed a selective reduction. It has been found that in compounds containing several metals not all of the metals are reduced simultaneously, but that the reducing action is sequential or successive depending upon the reactive energy required to split the compounds into their elements, such, for instance, as reducing oxides into metal and oxygen, chlorides into metal and chlorine, etc. The reducing or reactive agent follows the lines of least resistance and acts upon the more responsive metallic compounds first, and the less responsive in sequence, so that if just sufficient **80** **85** **90** **95** **100** **105**

quantity of the reducing agent is supplied to the bulk of ore or metalliferous compounds to be treated to effect the desired reaction with the more responsive metals, 5 these latter will be reduced to metallic state before any material reducing action takes place between the reducing agent and the less responsive metallic values or other impurities, which it is desired to exclude from 10 the ultimate product, so that the desired metallic values, either in the form of a single metal, or an alloy of metals, may be recovered with only a relatively small proportion of the impurities or undesirable elements admixed therewith and which are 15 not sufficient to impair the commercial value of the final product, the major portion of the impurities remaining in the slag and being carried off therewith.

20 For example, it has been found that tungstic oxide and iron oxide are readily reduced and when reduction is effected by the aluminothermic method these two oxides will be reduced to ferro-tungsten before any 25 appreciable amount of the other oxides usually found in ores and compounds containing these metals, such as silica and manganese oxide, are attacked, and, by regulating the quantity of aluminum employed to 30 just sufficient to reduce all of the tungsten and iron compounds present, the reducing operation will be suspended when this result has been effected, and most of the silica and manganese will remain in the slag. Of 35 course, it is not feasible to reduce all of the tungstic oxide and iron oxide in an ore or compound before any of the remaining metallic compounds begin to react with the aluminum, but I have found that it is possible to effect a reduction of 80% of the 40 tungstic oxide in the reduction mixture before as much as 10% of the silica and manganese oxide has reacted. It is therefore possible to reduce tungsten ores containing as high as 7% manganese oxide and 45 7% silica by means of the aluminothermic reaction, and still produce a very high ferro-tungsten alloy which contains considerably less than 1% manganese and 1% silicon, 50 an amount which is permissible in the trade.

55 It is obvious that in reducing an ore or compound so high in impurities the recovery in metallic tungsten is fractionally lower than in the case of pure raw material, such as tungstic oxide or calcium tungstate, but the loss is very small and amounts to only a fraction of the cost of any effective preparatory treatment of the ore to eliminate the impurities before the reduction is 60 effected.

65 In order to arrive at the proper proportions of the reducing agent to be employed, it is essential to know the various constituents of the ore or compound and then to regulate the quantity of the reducing agent,

relative to the amounts or proportions of the desired metal or metals. For example, if the proportions by weight of tungstic oxide and iron oxide in a given ore or mixture are known, the amount of aluminum 70 required to produce a satisfactory recovery of ferro-tungsten may be readily arrived at either by calculation or by running a test on a small proportion of the compound or ore, the results of which will indicate at 75 once whether the resultant ferro-tungsten is satisfactory and sufficiently low in impurities to be commercially acceptable. After this condition has been established and the proper proportion of the reducing 80 agent determined, the entire lot of ore from which the test sample was taken, is reduced under the same conditions. All operations, except the preparation of the reduction mixture, are carried out in the same manner 85 as the usual aluminothermic reactions for the recovery of metallic values, with the assurance that the resultant ferro-tungsten alloy will contain only permissible proportions of the objectionable elements, such as silicon and manganese. All other impurities, 90 such as phosphorus, sulphur, etc., may be present within the same limitations as are required for the production of ferro-tungsten in the electric furnace or for the production of tungsten powder by means of the 95 alkali fusion process.

The success and efficiency of the method as described may be illustrated by taking a concrete example of one of the well known 100 tungsten ores containing the following percentage of metallic oxides:

|                  | Per cent. |     |
|------------------|-----------|-----|
| WO <sub>3</sub>  | 69.02     | 105 |
| SiO <sub>2</sub> | 3.13      |     |
| MnO              | 7.50      |     |
| FeO              | 21.39     |     |

and treating successive batches thereof by the aluminothermic method, the first reaction involving sufficient aluminum to reduce all of the oxides present, the second batch being treated with a lesser amount of aluminum which would leave some of the impurities or undesirable oxides unreduced, 110 and the third producing a ferro-tungsten in which the proportions of manganese and silicon were well within the permissive commercial limits.

In the first case, 25.25 pounds of aluminum per 100 pounds of ore were used and an analysis of the alloy showed the following proportions:

|           | Per cent. |     |
|-----------|-----------|-----|
| Tungsten  | 70        | 125 |
| Iron      | 21        |     |
| Silicon   | 1.8       |     |
| Manganese | 7.2       |     |

Such an alloy would probably have a very limited application in the trades, because 130

of the relatively high percentages of the impurities or objectionable elements silicon and manganese.

In the second run 21.5 pounds of aluminum per 100 pounds of ore were used and the analysis showed the following proportions of metallic constituents in the resultant alloy:

|             | Per cent. |
|-------------|-----------|
| 10 Tungsten | 78        |
| Iron        | 17        |
| Silicon     | 1.13      |
| Manganese   | 2.23      |

15 This clearly demonstrates that one of the objectionable impurities, to wit, manganese, has been partially eliminated. This was accompanied, of course, by a slight loss in efficiency in the tungsten content recovery.

20 In the third case, 21 pounds of aluminum per 100 pounds of ore were used and the resultant alloy showed tungsten 78%, iron 19%, silicon 0.8%, manganese 0.32%, in which the proportions of silicon and manganese are well within permissive limits and the product being an alloy not limited in its use because of the presence of impurities. This last result was accomplished without any material loss in the efficiency of the 30 tungsten recovery.

It will therefore be apparent that, by employing the aluminothermic method of reduction in connection with the particular ore referred to, it was possible to eliminate a 35 very large proportion of the objectionable elements without any of the ordinary preliminary treatment required in connection with ores of this general character and to produce a commercially acceptable ferro-tungsten direct from the ore. It will also 40 be apparent that, by properly selecting and apportioning the amount of the reducing agent employed, a very wide range of ores may be treated to produce ferro-tungsten 45 of the same degree of purity, and the process is, therefore, not limited to ores which are carefully selected as would be the case

even when the latter are subjected to preliminary treatment, preparatory to reduction of high grade metals and alloys.

60

It is to be understood, of course, that the invention is not limited to the use of aluminum only as the reducing agent, as it is possible to employ other reducing agents and combinations of aluminum and other 55 reducing agents, provided that the proportions of the reducing agent or agents employed be so regulated, with respect to the metal or metals to be recovered, that the reducing action will be confined largely between the desired metallic values and the 60 reducing agent and the action of the latter on the undesired elements will be so limited that the proportions of the impurities in the resultant metal or alloy reduced will be unimportant.

What I claim is:

1. The method of producing metals or alloys from compounds comparatively high in impurities, which comprises effecting the 70 aluminothermic reaction in the compound, and so regulating the amount of aluminum as to substantially restrict the reducing action to the desired metalliferous material.

2. The method of producing ferro-tungsten from compounds comparatively high in impurities, which comprises effecting a reaction between the compound and a reducing agent, and so regulating the amount of said reducing agent as to substantially restrict 80 the reaction to the reduction of the iron and tungsten.

3. The method of producing ferro-tungsten from compounds comparatively high in impurities, which comprises effecting the 85 aluminothermic reaction in the compound, and so regulating the amount of aluminum as to substantially restrict the reducing action to the iron and tungsten.

Signed at Jersey City, in the county of 90 Hudson and State of New Jersey, this 19th day of November A. D. 1919.

CARL ROBERT SCHROEDER.